

Patented Dec. 29, 1936

2,065,534

# UNITED STATES PATENT OFFICE

2,065,534

## PROCESS FOR IMPROVING ALUMINUM ALLOY

Alfred J. Lyon, Dayton, Ohio

No Drawing. Original application April 7, 1930,  
Serial No. 442,468. Divided and this applica-  
tion July 5, 1934, Serial No. 733,861

9 Claims. (Cl. 75—140)

(Granted under the act of March 3, 1883, as  
amended April 30, 1928; 370 O. G. 757)

The invention described herein may be manufactured and used by or for the Government for governmental purposes, without the payment to me of any royalty thereon.

5 My invention relates to the improvement of aluminum alloys containing copper as the principal alloying constituent with other elements in lesser amounts such as nickel, iron, silicon, magnesium, chromium, lithium, calcium or manganese or any combination of these elements.

One object is to provide alloys of this type for use in cast and wrought parts, having improved physical properties, especially tensile strength, elongation and hardness; another object is to improve the soundness and eliminate porosity in alloys of this type used in the form of castings that must resist pressure such as cylinder heads and other parts of internal combustion engines; a further object is to provide a method of producing these improvements in a simple and inexpensive manner.

20 Aluminum copper alloys are known to be divided into two groups. The first group comprises those alloys containing from three to six per cent copper and includes numerous compositions used commercially in both the wrought and cast condition with and without heat treatment. The other group comprises those alloys containing greater than six per cent copper and are used commercially in the cast condition with or without heat treatment.

25 My invention is based on the discovery that all or a part of the alloying constituents of aluminum base alloys may be incorporated into the alloys by the means of their chloride compounds thereby greatly affecting the hardness, strength, ductility and soundness of castings or parts made from these alloys in accordance with methods well known to the art. The effect upon the physical properties varies with the chloride compound used and the copper content which may vary from three to fifteen per cent, and the properties that are obtained are different than the properties that are obtained when the metal of the chloride compound is incorporated into the alloy by the usual and known methods. I am aware that certain chlorine compounds have been used as fluxes in connection with the melting of aluminum alloys for the purpose of cleansing the metal from impurities. My invention of course is not primarily concerned with this phase of aluminum alloy treatment, altho I recognize that in the treatment of aluminum alloys in accordance with my invention this cleansing is incidental to the modifying "effect" or grain refining that the compounds have upon the alloy. For example the compound NH<sub>4</sub>Cl is well known to have a cleansing effect upon aluminum and other alloys but does not

produce a "modifying effect" as is illustrated by the following results:

Chemical composition: Copper—4.3 per cent, silicon—0.7 per cent, iron—0.5 per cent

|                                    | Tensile strength, lbs. per sq. in. | Elongation, 2 ins. percent | Brinell hardness | 5  |
|------------------------------------|------------------------------------|----------------------------|------------------|----|
| With 0.5 percent ammonium chloride | 32,400                             | 3.7                        | 76               | 10 |
| With no additions                  | 35,800                             | 4.7                        | 80               |    |

Likewise ZnCl<sub>2</sub> and NaCl are used in small amounts for the same purpose without any modifying effect.

15 United States Patent Number 1,676,856 to Alfred George Cooper Gwyer and Henry Wilfred Lewis Phillips of London, England, discloses the fact that the tensile strength and ductility of the aluminum-copper alloys can be increased, and the grain structure refined, by the addition of the alkaline earth metals, barium, strontium or calcium. I am aware that the alkaline earth metal hydroxides, alkaline earth metals, fluorides, 20 sodamide and the oxide compounds of the alkaline earth metals when introduced into aluminum alloys containing more than six per cent copper, in the molten condition have a modifying effect and increase the strength, hardness and ductility 25 of castings made from these alloys. I am also aware that the alkaline earth metals, their fluoride, oxide and hydroxide compounds and certain other metals such as bismuth, antimony, boron and manganese are known to improve the strength 30 and ductility of aluminum alloys containing substantial amounts of silicon as the principal alloying constituent when added to the molten alloy. I have found by a series of tests upon aluminum alloys containing three to six per cent copper as 35 the principal alloying constituent and with small amounts of iron and silicon as impurities that metals and elements that "modify" and refine the grain structure of aluminum copper alloys containing more than six per cent copper or aluminum alloys containing from three to fifteen 40 per cent silicon as the principal alloying constituent, do not have the same effect upon alloys of the type which are included in my invention. As an illustration I have added metallic sodium, potassium, potassium fluoride, sodium fluoride or lithium fluoride to aluminum copper alloys containing four per cent copper without improving the strength, ductility or hardness, but when I added lithium chloride in the same manner and 45 in the same amounts to the molten alloy I obtained substantial improvements in the strength and ductility of the alloy when cast under the same conditions as the untreated alloy. This is 50 in accordance with the known facts concerning 55 60

the modification of aluminum alloys for the purpose of refining the grain structure and improving the physical properties. What happens in the case of aluminum-silicon, aluminum-iron, or aluminum-copper alloys of one class is no guide to what happens in the case of other alloys.

I am aware that aluminum is a metal frequently used as a reducing agent in processes involving the reduction of oxides of metals. The "Thermite" process invented by Goldsmith is an example in which metallic oxides are reduced by aluminum. I have incorporated manganese for example into aluminum copper alloys by this principle by using the compound manganese dioxide but it has no "modifying" effect when added in this manner.

In the preferred practice of the present invention, a copper-aluminum alloy is prepared in the usual manner by melting aluminum ingot which 20 contains small amounts of iron and silicon as impurities, together with the copper and all or a part of other alloying constituents in the form of commercially pure metals or in the form of rich alloys of the alloying constituents with aluminum. 25 When the alloy is molten and has reached a temperature of approximately 700 degrees centigrade, I introduce the chloride compound of one or more of the alloying constituents as described herein-after.

30 Chloride compounds are hydroscopic and before introducing them to the molten aluminum, they must be dried by heating to a temperature of approximately 100° C. for several hours and then crushed to break down lumps and crusts that form 35 during the drying treatment, or they may be melted and poured into sticks or other forms of convenient size for introducing into the molten metal.

The chlorides are then incorporated with the 40 molten aluminum alloy by wrapping weighed quantities in aluminum foil or paper and holding it beneath the surface of the molten metal. For this purpose a section of wrought iron pipe open at both ends is welded to an iron rod or handle, 45 in such a manner that the section of pipe, approximately 4 inches in length and 1½ inches in diameter, may be lowered beneath the surface of the molten metal in a horizontal position. The chloride compounds in this manner are held beneath the surface of the metal until the reaction 50 is completed. Stirring or agitation of the metal by mechanical means is not necessary as the reduction of the chlorides is accompanied by considerable agitation of the metal with an evolution 55 of chlorine gas.

The chloride compounds can also be incorporated into the aluminum or aluminum alloys by other methods, such as pouring the molten metal into a crucible pre-heated with the chloride compound 60 pounds in the bottom, or by stirring the powdered and dried salts into the molten metal. However, these methods do not produce as satisfactory results and I prefer to use the method first described.

65 I have found that certain of the metal chlorides added to the aluminum alloys in the molten condition in accordance with this method caused an improvement in physical properties, but when remelted without further addition of these chlorides, 70 the gained strength, hardness and ductility are partially lost and in some instances cause the properties to be inferior to the untreated alloy. As an illustration, the following results were obtained on standard test specimens cast from an 75 alloy containing 4.3 percent copper, 0.5 percent

iron, and 0.7 percent silicon, in green sand and heat treated by a method well known to the art.

| Chloride added | Percent | Tensile strength PSI | Elongation in 2 ins. percent | Brinell hardness | Remarks                                                                 | 5  |
|----------------|---------|----------------------|------------------------------|------------------|-------------------------------------------------------------------------|----|
| Copper         | 0.25    | 37,300               | 7.5                          | 79               | As treated.<br>1st remelt.<br>2nd remelt.                               |    |
|                | Do      | 36,490               | 7.5                          | 77               |                                                                         | 10 |
|                | Do      | 34,720               | 6.3                          | 76               |                                                                         |    |
| Iron           | 0.25    | 38,600               | 8.0                          | 80               | As treated.<br>1st remelt.<br>2nd remelt.                               |    |
|                | Do      | 36,970               | 7.7                          | 76               |                                                                         |    |
|                | Do      | 34,580               | 6.3                          | 74               |                                                                         |    |
| Zinc           | 0.25    | 35,900               | 7.3                          | 75               | As treated.<br>1st remelt.<br>2nd remelt.                               |    |
|                | Do      | 37,650               | 9.2                          | 77               |                                                                         |    |
|                | Do      | 32,950               | 6.5                          | 72               |                                                                         | 15 |
| Manganese      | 0.25    | 40,820               | 7.2                          | 85               | As treated.<br>1st remelt.<br>2nd remelt.<br>As treated.<br>1st remelt. |    |
|                | Do      | 40,760               | 5.5                          | 88               |                                                                         |    |
|                | Do      | 42,140               | 5.0                          | 90               |                                                                         |    |
|                | 0.50    | 44,080               | 8.0                          | 90               |                                                                         |    |
|                | Do      | 42,820               | 7.5                          | 86               |                                                                         |    |
| Nickel         | 0.25    | 38,367               | 8.0                          | 78               | As treated.<br>1st remelt.<br>2nd remelt.<br>As treated.<br>1st remelt. | 20 |
|                | Do      | 36,560               | 7.0                          | 78               |                                                                         |    |
|                | Do      | 36,400               | 7.0                          | 78               |                                                                         |    |
|                | 0.50    | 40,630               | 9.0                          | 80               |                                                                         |    |
|                | Do      | 39,400               | 9.0                          | 81               |                                                                         |    |
| Tin            | 0.25    | 52,250               | 1.0                          | 123              | As treated.<br>1st remelt.<br>2nd remelt.                               |    |
|                | Do      | 50,500               | 0.7                          | 121              |                                                                         | 25 |
|                | Do      | 47,700               | 0.8                          | 118              |                                                                         |    |
| Chromium       | 0.25    | 41,000               | 9.0                          | 80               | As treated.<br>1st remelt.<br>2nd remelt.                               |    |
|                | Do      | 39,100               | 8.5                          | 81               |                                                                         |    |
|                | Do      | 37,700               | 7.5                          | 80               |                                                                         |    |
| Lithium        | 0.50    | 38,400               | 8.8                          | 77               | As treated.<br>1st remelt.<br>2nd remelt.                               | 30 |
|                | Do      | 39,550               | 10.3                         | 78               |                                                                         |    |
|                | Do      | 40,300               | 11.0                         | 80               |                                                                         |    |
| None           |         | 36,910               | 5.6                          | 82               | As mixed.<br>1st remelt.                                                |    |
|                | Do      | 37,525               | 7.5                          | 80               |                                                                         |    |

By adding certain of the metal chlorides in additional amounts upon remelting the properties of the alloy can be improved and restored to values equal to or greater than those obtained by the first addition of the metal chloride. Nickel, lithium and copper chlorides are especially useful for this purpose, but further additions of iron, zinc, chromium, or tin chlorides adversely affect the strength and hardness. This is illustrated by the results tabulated in the following table, obtained on standard specimens cast in sand and heat treated from an aluminum alloy containing 4.3 per cent copper and small amounts of silicon and iron.

| Chloride added | Percent | Tensile strength PSI | Elongation in 2 ins. percent | Brinell hardness | Remarks                                                  | 50 |
|----------------|---------|----------------------|------------------------------|------------------|----------------------------------------------------------|----|
| Nickel         | 0.25    | 38,367               | 8.0                          | 78               | 1st remelt.<br>2nd remelt.<br>3rd remelt.<br>4th remelt. |    |
|                | 0.25    | 40,630               | 9.0                          | 80               |                                                          |    |
|                | 0.50    | 39,400               | 9.0                          | 81               |                                                          |    |
|                | 0.50*   | 38,980               | 10.0                         | -----            |                                                          |    |
| Copper         | 0.25    | 37,300               | 7.5                          | 79               | 1st remelt.<br>2nd remelt.<br>3rd remelt.<br>4th remelt. |    |
|                | 0.25    | 38,450               | 8.7                          | 80               |                                                          |    |
|                | 0.50    | 37,050               | 7.3                          | 79               |                                                          |    |
|                | 0.50*   | 41,830               | 11.0                         | 82               |                                                          | 60 |
| Zinc           | 0.25    | 35,900               | 7.3                          | 75               | 1st remelt.<br>2nd remelt.<br>3rd remelt.<br>4th remelt. |    |
|                | 0.25    | 37,350               | 9.5                          | 74               |                                                          |    |
|                | 0.50    | 35,880               | 9.0                          | 74               |                                                          |    |
|                | 0.50*   | 33,020               | 7.7                          | 73               |                                                          |    |
| Tin            | 0.25    | 52,250               | 1.0                          | 123              | 1st remelt.<br>2nd remelt.<br>3rd remelt.<br>4th remelt. |    |
|                | 0.25    | 37,875               | 0.5                          | 122              |                                                          |    |
|                | 0.50    | 36,500               | 0.5                          | 119              |                                                          |    |
|                | 0.50*   | 27,250               | -----                        | 117              |                                                          |    |
| Chromium       | 0.25    | 40,850               | 9.0                          | 81               | 1st remelt.<br>2nd remelt.<br>3rd remelt.<br>4th remelt. |    |
|                | 0.25    | 37,100               | 6.0                          | 80               |                                                          |    |
|                | 0.50    | 36,050               | 5.0                          | 79               |                                                          |    |
|                | 0.50*   | 36,700               | 6.0                          | 81               |                                                          | 70 |

\*Total chloride adding in process of remelting equals 1.5 percent.

In carrying out my invention in the preferred manner, it may be seen in the foregoing that specific amounts of the chloride compound must

be used to obtain the optimum physical properties of castings or parts made from the alloy. As further specific example, the following tabulation in Column "B" illustrates the effect and physical properties of adding increasing amounts of manganese by means of manganese chloride to the alloy containing 4.3 percent copper, 0.69 percent silicon and 0.51 percent iron. The manganese incorporated into the alloy was determined by chemical analysis to be  $\frac{2}{5}$  of the weight of its chloride compound.

| 15 | Man-ganese, percent | Tensile strength, lbs. per sq. in. |        |        | Elongation in 2", percent |      |     | Brinell hardness |    |    |
|----|---------------------|------------------------------------|--------|--------|---------------------------|------|-----|------------------|----|----|
|    |                     |                                    |        |        |                           |      |     |                  |    |    |
|    |                     | A                                  | B      | C      | A                         | B    | C   | A                | B  | C  |
| 20 | 0.05                | 34,850                             | 42,510 | 36,150 | 6.7                       | 7.5  | 4.3 | 77               | 89 | 80 |
|    | 0.10                | 31,650                             | 45,810 | 34,470 | 6.7                       | 10.6 | 7.2 | 73               | 89 | 73 |
|    | 0.20                | 32,480                             | 40,100 | 29,670 | 7.8                       | 7.8  | 4.8 | 71               | 94 | 70 |

The results shown in Columns "A" and "C" are for the purpose of illustrating the improved properties I obtain by using the chloride compound, since it is well known to the art that the method of casting and the type of specimen has a profound effect on the physical properties. The results in Columns "A", "B" and "C" were obtained 25 upon the same type test specimens, sand cast and heat treated in the same manner. The manganese was incorporated into the alloy from which the results in Column "A" were obtained by the usual method of using a manganese rich 30 alloy containing 10 percent manganese and approximately 90 percent aluminum. The manganese was incorporated into the alloy, from which the results in Column "C" were obtained by means of manganese dioxide added to the 35 molten alloy before pouring. I have found that the best results for a manganese chloride modified alloy of this type are obtained when manganese chloride is used in the amounts from about .4 to .5 per cent.

45 As another example of improving the properties of eliminating the defects from certain alloys of the type that are the subject of my invention, such as eliminating porosity, I melt an aluminum alloy containing 4 percent copper, 1 $\frac{1}{2}$  percent magnesium, and 2 percent nickel in the usual manner and when the molten metal has reached a temperature of 700° C., I introduce nickelous chloride or cupric chloride or a mixture of nickelous and cupric chlorides in amounts greater than .75 per cent. (Less than .7 per cent nickelous chloride does not produce the result desired.) Other chloride compounds may be used for this purpose, but where zinc is used, for example, the strength of the alloy at high temperature is 50 adversely affected.

By introducing the chloride compounds of lithium or manganese or a combination thereof into the molten alloy in the manner already described and preferably in amounts from about .25 per cent to 1 per cent, the grain structure and the size of the particles of the alloying constituents are reduced and refined and consequently go into solid solution more quickly thus shortening the period of the usual heat treatment.

70 The alloys produced according to my invention may be utilized for any kind of casting, and such castings may be worked as by rolling, extruding, forging, drawing, etc. The results quoted for physical properties are based upon sand cast specimens and do not represent the maximum

physical properties obtainable in castings or the properties of the materials in the wrought condition. It is well known that the tensile properties of cast alloys are greatly improved by casting in metal molds or by chilling and that the strength and hardness of a chill casting is increased to a marked degree by rolling or forging. 5

From these and other experiments, I have discovered that each of the chloride compounds added to the molten aluminum alloy of this type 10 affect the physical properties of the heat treated castings in a manner that cannot be obtained by the addition of the metal of the compound; by the reduction of other compounds containing the metal by the addition of metal in the primary 15 state; or by treating the metals with chlorine gas obtained by the reduction of such compounds as ammonium chloride.

Therefore, in carrying out my invention in the preferred manner, I select one of the chloride 20 compounds or a mixture of two or more chloride compounds that produce the special combination of properties such as strength, hardness or strength and ductility and soundness that may be required in the part or casting made from the 25 alloy.

This application is a division of application Serial No. 442,468, filed Apr. 7, 1930, which has issued as Patent No. 1,965,604, dated July 10, 1934.

I claim:

1. A process for producing aluminum-copper alloy, which consists in the steps of melting together a mixture consisting predominately of aluminum and containing 3% to 15% copper as the 35 principal alloying constituent, and thereafter incorporating in the molten alloy a material containing tin chloride.

2. A process for producing aluminum-copper alloy, which consists in the steps of melting together a mixture consisting predominately of aluminum, copper 3% to 15%, and iron and silicon in lesser amounts and thereafter incorporating a material containing tin chloride in the molten alloy at a temperature of about 700° centigrade. 45

3. A process for producing aluminum-copper alloy, which consists in the steps of melting aluminum containing iron about .5% and silicon about 7%, together with copper about 4.3%, and thereafter introducing into the molten alloy a 50 chloride of tin in a relatively limited amount.

4. A process for producing aluminum-copper alloy, which consists in the steps of melting aluminum containing iron about .5% and silicon about 7%, together with copper about 4.3%, and 55 thereafter adding to said molten alloy about .25% tin chloride.

5. A process of producing an aluminum-copper alloy which consists in the steps of melting together a mixture consisting predominately of 60 aluminum containing 3% to 15% copper as the principal alloy constituent and thereafter incorporating a material containing tin chloride into said molten alloy at a temperature of about 700° centigrade. 65

6. A process of producing an aluminum-copper alloy which consists in the steps of melting together a mixture consisting predominately of aluminum containing 3% to 15% copper as the principal alloy constituent and thereafter incorporating a chloride of tin in a relatively limited amount into said molten alloy at a temperature of about 700° centigrade. 70

7. A process of producing an aluminum-copper 75

alloy which consists in the steps of melting together a mixture consisting predominately of aluminum containing 3% to 15% copper as the principal alloy constituent and thereafter incorporating about .25% tin chloride to said alloy at a temperature of about 700° centigrade.

8. A process of producing an aluminum-copper alloy which consists in the steps of melting together a mixture consisting predominately of aluminum containing 3% to 15% copper as the principal alloy constituent and thereafter incorporat-

ing a dehydrated material containing tin chloride into said molten alloy.

9. A process of producing an aluminum-copper alloy which consists in the steps of melting together a mixture consisting predominately of aluminum containing 3% to 15% copper as the principal alloy constituent and thereafter incorporating a dehydrated material containing tin chloride into said molten alloy at a temperature of about 700° centigrade. 5

ALFRED J. LYON. 10